

Dec. 15, 1964

J. J. SCOTT

3,161,472

ARC FURNACE PROCESS FOR THE PRODUCTION OF TITANIUM CARBIDE

Filed Feb. 25, 1958

5 Sheets-Sheet 1



Fig. 2



Fig. 4



Fig. 5

INVENTOR  
JOHN J. SCOTT  
BY  
*John J. Scott*  
ATTORNEY

Dec. 15, 1964

J. J. SCOTT

3,161,472

ARC FURNACE PROCESS FOR THE PRODUCTION OF TITANIUM CARBIDE

Filed Feb. 25, 1958

5 Sheets-Sheet 2

Fig. 10



Fig. 9



Fig. 11

Fig. 8



JOHN *J. SCOTT* INVENTOR

BY

ATTORNEY

Dec. 15, 1964

J. J. SCOTT

3,161,472

## ARC FURNACE PROCESS FOR THE PRODUCTION OF TITANIUM CARBIDE

Filed Feb. 25, 1958

5 Sheets-Sheet 3



Fig. 12

JOHN J. SCOTT INVENTOR

BY

Franklin Roosevelt

ATTORNEY

Dec. 15, 1964

J. J. SCOTT

3,161,472

ARC FURNACE PROCESS FOR THE PRODUCTION OF TITANIUM CARBIDE

Filed Feb. 25, 1958

5 Sheets-Sheet 4



Fig. 13

INVENTOR  
JOHN J. SCOTT

BY

*George Donisthorpe*  
ATTORNEY

Dec. 15, 1964

J. J. SCOTT

3,161,472

ARC FURNACE PROCESS FOR THE PRODUCTION OF TITANIUM CARBIDE

Filed Feb. 25, 1958

5 Sheets-Sheet 5



*Fig. 14*

INVENTOR  
*John J. Scott*

BY *Reuben M. Franklin*  
ATTORNEY

1

3,161,472

**ARC FURNACE PROCESS FOR THE PRODUCTION  
OF TITANIUM CARBIDE**

John J. Scott, Willoughby, Ontario, Canada, assignor to  
Norton Company, Worcester, Mass., a corporation of  
Massachusetts

Filed Feb. 25, 1958, Ser. No. 717,494  
4 Claims. (Cl. 23—208)

The invention relates to the production of titanium carbide.

One object of the invention is to reduce the cost of synthesizing titanium carbide. Another object of the invention is to provide a practical process for synthesizing titanium carbide from readily available titaniferous ores such as rutile, and titania slag. Titania slag is a by-product resulting from the extraction of iron content from certain ilmenite ores, for example such as found in the Province of Quebec.

Another object of the invention is to synthesize titanium carbide especially suitable for the extraction of titanium metal by means of an electrolytic process using a fused salt bath such as disclosed, for example in a co-pending application of my colleagues Guy Ervin, Jr., and H. F. G. Ueltz, Serial No. 394,753, filed November 27, 1953, now abandoned.

Another object of the invention is to provide a process of the type indicated which will readily eliminate the silica content, the alumina content and iron content of the titaniferous ore as well as other compounds or elements occurring therein in minor percentages. Another object of the invention is to produce high purity titanium carbide in particle sizes suitable for the manufacture by sintering or the like of crucibles, cells or other bodies useful for the production of titanium metal or otherwise in an arc furnace operation without the necessity of further treatments such as washing or crushing to fines. Another object is to produce a titanium carbide suitable for the extraction of titanium metal by various processes. Another object is to avoid contamination of the carbide product produced. Another object is to reduce the volume of molten carbide present at any given time in the furnace available for contamination by air.

Another object is to produce titanium carbide having a content of desirable metal such as chromium, niobium, zirconium and/or vanadium for the ultimate production of titanium metal alloyed with such metal or metals.

This application is a continuation in part of by co-pending application Serial No. 455,920, filed September 14, 1954, now abandoned.

Other objects will be in part obvious or in part pointed out hereinafter.

In the accompanying drawings illustrating one type of arc furnace by means of which the process of the invention can be carried out,

FIGURE 1 is a front elevation of the furnace shell,

FIGURE 2 is a plan view of the furnace shell,

FIGURE 3 is a sectional view of the furnace shell, the section being taken along the line 3—3 of FIGURE 1,

FIGURE 4 is a sectional view of the wall of the furnace shell, the section being taken along the line 4—4 of FIGURE 2,

FIGURES 5 and 6 are fragmentary sectional views taken on the lines 5—5 and 6—6 respectively of FIGURE 1,

FIGURES 7 and 8 are plan views of water-cooling pipes,

FIGURE 9 is a front elevation of a furnace bottom truck,

2

FIGURE 10 is a plan view of the furnace bottom truck,

FIGURE 11 is a sectional view taken along the line 11—11 of FIGURE 9,

FIGURE 12 is a front elevation of the furnace completely assembled, illustrating the carbon or graphite electrodes and the track upon which the wheels of the truck rest,

FIGURE 13 is a graph showing the operating conditions for the furnace described,

FIGURE 14 is a diagrammatic elevational view of the arc furnace in operation producing separate ingots of carbide material under each electrode.

Referring now to FIGURES 1, 2, and 3, the furnace shell 20 can be made out of two pieces of steel plate welded together. Its shape is oval, tapering from the bottom to the top, and the shape is sufficiently indicated in FIGURES 1, 2 and 3. As shown in FIGURES 1, 4 and 5 at the top of the shell 20 is welded a lip 21 to which is welded a depending skirt 22. At the bottom of the shell 20 is a large flange 23, which also can be made of steel plate and welded to this flange 23 is a depending skirt 24. As clearly shown in FIGURE 3 the outer contour of the flange 23 is circular while the inner contour is oval; the flange 23 is welded to the shell 20. Steel ribs 25, 26, 27, and 28 are welded to the shell 20 and to the flange 24 and serve to give this unit great strength.

Hooks 30 made of steel plate are welded to the outside of the shell 20, near the top, at opposite ends of the long axis of the oval. These hooks 30 can be engaged by the hooks of chain falls connected to an overhead hoist, not shown, for the purpose of lifting the unit comprising the shell off the product of the fusion when the latter has cooled sufficiently.

A pair of bent pipes 32, one of which is shown in FIGURE 7 and the other of which is identical therewith except that it is of the opposite hand, are provided with very fine holes 33 which are preferably located (when the pipes 32 are in place as shown in FIGURES 4 and 5) to throw water upwardly and inwardly; for example they can be 30° from the top and on the inside as illustrated. At one end of each pipe 32 is a pair of elbows 34 and 35 connected to each other and to a nipple 36. At the other end of each pipe 32 is a cap 37 to plug the free end of the pipe whereby to compel the water to issue through the holes 33. The pipes 32 can be supported under the lip 21 in any manner; as illustrated in FIGURES 2 and 5 it will suffice to provide four bolts 40 extending through the lip 21 upholding bars 41 by means of nuts 42, and the pipes 32 simply rest upon the bars 41.

FIGURE 8 illustrates one of a pair of bent pipes 45, of which one is as shown and the other is of the opposite hand, and these pipes 45 have holes 46 and are equipped with elbows 47 and 48 and a connecting nipple 49 on one end, and caps 50 on the other end. As shown in FIGURES 1 and 6 these pipes can be supported close to the shell 20 by means of lugs 52 welded to the outside of the shell 20 together with bent bolts 53 passing through pipe sleeves 54 welded to the lugs 52, and with nuts 55 to draw the bent bolts firmly against the pipes 45. Illustratively the holes 46 can be oriented as shown in FIGURE 6, but this is not critical so long as they are located to throw the water inwardly since at the locus of pipe 45 there is already a cascade of water.

The pipes 32 and 45 are, of course, connected to water supply as by means of hoses 57, 58, 59, and 60 illustrated in FIGURE 12, so that at all times when the power is on, the shell 20 is cooled by a cascade of water. Although

the synthesis of titanium carbide takes place at about 3000° C. and above and steel plate melts at around 1500° C., the cascade of water over the shell 20 coupled with the fact that steel is highly thermally conductive protects the shell 20 from melting. The cascade of water hugs the surface of the shell 20 and covers all parts of it from the top down and is assisted in so doing by the taper of the shell. Also it may be remarked that the shell 20 quickly acquires a coating of rust, which is easily understood since it is alternately wet and dry and frequently quite hot, and the rust makes it much more wettable than clean, un-rusted steel.

Referring now to FIGURES 9 and 10, the furnace bottom truck comprises a circular table 65 made of steel plate to which is welded a depending skirt 66 also made of steel plate. To the upper surface of table 65 is welded an oval bottom container 67 made of steel plate. This oval bottom container 67 has the same shape as the bottom of the shell 20 as shown in FIGURE 3, but the oval container 67 is slightly smaller in size so that the shell 20 and flange 23 can be placed over the container 67 and on the table 65. As shown in FIGURE 12, when the shell 20 is placed on the bottom with the flange 23 on the table 65, a hose 69 is interposed to act as a seal. This hose 69 is a plain piece of rubber hose without couplings or other fittings and simply acts as a cushion and sealing means, and extends all the way around the table 65 with the ends thereof overlapping.

Referring now to FIGURES 9 and 11 a pair of parallel steel I beams 70 are welded to the bottom of the table 65 and a plurality of I beams 71, for example three of them, are also welded to the bottom of the table 65. These I beams 71 are desirably perpendicular to the I beams 70. To the outer I beams 71 are welded U-shaped bars 72, for the purpose of connecting a hook of a chain to the truck to draw it along the track 73 illustrated in FIGURE 12.

Resting upon the track 73 are four flanged wheels 75 on steel axles 76 journaled in bearing boxes 77 which can be iron castings. The wheels 75 are located between the bearing boxes 77 and collars 78 on the axles 76. The bearing boxes 77 are welded to the under sides of the steel I beams 70.

Practical dimensions for the furnace described are, height of shell 20 about nine feet, other dimensions in proportion, and such a furnace can hold about 14,000 pounds of mixture and titanium carbide made therefrom.

A typical analysis of rutile ore, which is titaniferous ore, is given in the following table.

TABLE I

| Compound or element:                         | Percentage by weight |
|----------------------------------------------|----------------------|
| FeO and/or $Fe_2O_3$ calculated as $Fe_2O_3$ | 2.33                 |
| $Al_2O_3$                                    | 0.58                 |
| $SiO_2$                                      | 1.22                 |
| $Cr_2O_3$                                    | 0.12                 |
| $B_2O_3$                                     | 0.001                |
| $Ni_2O_3$                                    | 0.005                |
| CaO                                          | 0.08                 |
| MgO                                          | 0.11                 |
| $Nb_2O_5$                                    | 0.10                 |
| $P_2C_5$                                     | 0.12                 |
| $SnO_2$                                      | 0.08                 |
| S                                            | 0.01                 |
| $V_2O_5$                                     | 0.49                 |
| $TiO_2$                                      | 93.40                |
| $ZrO_2$                                      | <sup>1</sup> 1.354   |
|                                              | 100.00               |

<sup>1</sup> By difference.

A typical titania slag from the Quebec Iron and Titanium Corporation of Sorel, Province of Quebec, analyzed as follows.

4  
TABLE II

| Compound or element:   | Percentage of weight |
|------------------------|----------------------|
| $TiO_2$                | 77.27                |
| $Al_2O_3$              | 6.72                 |
| MgO                    | 5.84                 |
| $SiO_2$                | 5.00                 |
| CaO                    | 0.24                 |
| Iron content, magnetic | 4.24                 |
|                        | 99.31                |

This analysis shows no  $ZrO_2$  which was probably present but undetermined.

I use for a charge in the electric arc furnacing operation a mixture of the titaniferous ore, coke and reclaim material from a previous furnacing operation if I have any on hand that I consider of sufficiently high grade. In a furnacing operation according to the invention there is much material which is not converted to titanium carbide or is only partially converted and this is what I call reclaim material. The unconverted material is called sweepings as it falls to the floor when the furnace shell 20 is removed and the partly converted material which is found sintered around the outside of the pig is called refuse. Titaniferous ore and the two reclaim materials are generically referred to as titanium oxide ore.

I provide such a quantity of coke that the free carbon content thereof will be sufficient completely to reduce the titanium oxide ore and to carbonize it to titanium carbide,  $TiC$ , and up to 100% excess free carbon, that is to say from the stoichiometric proportion for such complete reduction and carbonization up to double such stoichiometric proportion. Thus I calculate the mass of the ore on hand including the reclaim material, and by atomic weights calculate the amount of carbon required to reduce and to carbonize the ore, then use this stoichiometric amount or additional carbon up to double the stoichiometric proportion. Of course the free carbon content of the coke is figured to find out the actual amount of coke to add. Free carbon content of coke determination is well known in the art and is done by analytical methods.

The theoretical amount of free carbon required to reduce  $TiO_2$  to  $TiC$  is 45% of the mass of the  $TiO_2$ , one third or 33.3% excess of carbon is 60% of the mass of the  $TiO_2$ , two thirds or 66.67% excess is 75% of the mass of the  $TiO_2$  and 100% excess of carbon is 90% of the mass of the  $TiO_2$ .

I prefer to use a well calcined coke principally because the amount of free carbon therein can be determined with more accuracy. I can use various kinds of coke, petroleum coke, metallurgical coke and pitch coke, but in general I find pitch coke is more uniform in quality and this usually has about 90% free carbon and is low in ash content, below 1%. I prefer to select coke having less than 5% ash content.

The titaniferous ore is intimately mixed with the coke and is further intimately mixed with the reclaim material. I can use coarse ore and/or coke or fine ore and/or coke, but the finer the particle sizes, the quicker and more complete is the reaction. The sweepings are used as they come, being fine material. The refuse is crushed to particles usually not larger than  $\frac{1}{4}$  inch lumps. The coke can be used as it comes, which is from  $\frac{1}{2}$  inch lumps to very fine particles. I can use 100% reclaim material (apart from the coke) or any proportion thereof relative to the total titaniferous material.

Before assembling the shell 20 and the bottom container 67, I form a carbon bottom in the container 67 in any suitable manner, such as by tamping in a mixture of fine carbon and pitch. This carbon bottom should be concave on the top and on the periphery should extend to the top of the container 67. After assembly of the shell 20 and bottom container 67, I pack reclaim material and/or ore between the outside of the container and the inside of the shell and then add more thereof to the shell

20 to extend to a rather uniform level about four inches above the top of the container 67 (assuming a nine foot high shell 20). This is also a bottom.

I now place a mass (for example about 75 pounds) of lump graphite or carbon right under the eventual loci of the electrodes 80 (see FIGURE 12) in which, when the furnace has been moved to operating position, are the foci of the oval of the shell 20. Electrically connecting these masses of carbon or graphite (termed carbon) I build a bridge of graphite or carbon with this lump material which bridge extends from one locus to the other locus. I form a trough in the reclaim material and/or ore for the lumps.

The bridge of graphite lumps forms a continuous electric current path from the area under one electrode to the area under the other electrode and the cross section of this path is preferably about fifty square inches for the large furnace described. Maximum and minimum permissible cross section of the bridge will be discussed hereinafter. I energize the electrodes 80 at an E.M.F. of from 50 to 150 volts, preferably 100 volts and then, having moved the truck on the track 73 to place the shell 20 in the proper position as above defined, I lower the electrodes into contact with the graphite. During the entire process the electric current flows through the bridge.

The electrodes are controlled by the usual overload-underload "servo" controlling mechanism and electric motor powered lifting and lowering mechanism, together with a circuit breaker to protect the electrical equipment. Since such electrical mechanisms are known and belong to an art other than the art of producing titanium carbide, they will not be described herein.

When the electrodes 80 contact the bridge of graphite, electric current flows at about 4000 amperes or more. The "servo" mechanism causes the electrodes 80 to hunt up and down maintaining the arcs with a current flow (when the E.M.F. is 100 volts) of about 8000 amperes.

Now I shovel mixture all over the area of the furnace to a depth of about two inches. Some mixture gets right into the loci of the arcs and there the reaction takes place, forming titanium carbide and releasing carbon monoxide. The conditions are reducing and the blanket of mix keeps the air away from the zone of reaction in the loci of the arcs. While it is preferable to have the blanket of mixture about one inch minimum depth at the electrodes and measuring from the bottoms of the electrodes in some cases I can operate without any blanket at all. Any blanket of mix should not be more than about three inches as I want the gases to escape.

It now suffices to charge the furnace from time to time with mixture. Away from the electrodes the mix should be banked high all around the inside of the shell 20. For example, it may be four inches higher at the shell than at the electrodes, and even higher, up to a foot higher at the ends of the long horizontal axis of the shell 20.

As mixture is fed from time to time into the furnace, the electrodes gradually rise as ingots of titanium carbide are formed in the loci of the arcs. No considerable pool of molten titanium carbide is formed; the reaction produces a titanium carbide which is incandescent and some liquid phase may exist but for the most part the liquid phase is momentary only.

The operation of the furnace part way through a run as described above is illustrated in FIG. 14, which shows the base layer 32 of ore, reclaim material or comparable material supporting the large lumps 84 and 84a of graphite or carbon under the loci of the electrodes 80. Between the carbon lumps 84 and 84a is the bridge of graphite or carbon lumps 86 and extending substantially between the bottom of each electrode 80 and the corresponding large carbon lump 84 or 84a are the fused ingots 88 and 88a of carbide material. Surrounding the bottom ends of the electrodes 80, ingots 88 and 88a and carbon bridge formed of lumps 84, 84a and 86 is the mass of reaction

mixture 90, which as exemplified above will rise higher and higher in the shell 20 as the production run proceeds. The path of electric current during the operation is from one electrode 80 via an arc 92, through the ingot 88, the lump 84, then the lumps 86, next the lump 84a, then the ingot 88a, and finally through the arc 92a to the other electrode.

When the run has been completed, and the electrodes lifted, it is convenient to draw the truck along the rails 10 73 to remove the entire furnace from under the electrodes so that, for example, another similar furnace may be set up underneath them to start another run of the process. However, for a long time the cascade of water is maintained on the shell 20, preferably at least through 15 the hoses 57 and 58 to the pipes 32. This cascade of water is maintained until the contents of the shell 20 has cooled sufficiently so that there is no more danger of burning the shell. Usually this takes about sixteen hours. The furnace shell is not lifted until the contents have 20 cooled sufficiently so that the carbide will not oxidize when it comes into contact with the air. In a 14,000 lb. furnace shell this is about 40 hours from the time the furnace is shut down. At the end of that time, the furnace shell is lifted off the ingots and what is now reclaim 25 material, which forms a loosely sintered mass. Two ingots of titanium carbide are found embedded in the mix. The ingots are carefully separated from what is now reclaimed material and the latter is collected for use in a subsequent run of the process.

30

#### EXAMPLE I

Using a furnace the shell 20 of which was 38 inches high instead of the furnace recommended, which 38 inch high shell will hold a maximum of about 1000 lbs. of this material, this one thousand pound furnace being, however, 35 of the same shape and proportions and having the same parts as the fourteen thousand pound furnace described, I synthesized thirty-six pounds of titanium carbide as follows:

40 The charge was 300 pounds of rutile and 200 pounds of pitch coke having a free carbon content of 90%. Thus the coke had one hundred eighty pounds of free carbon which is 60% of the mass of the rutile which was so nearly pure  $TiO_2$  that I disregarded the difference. The 45 actual analysis of this rutile was as follows.

| Compound:          | Percentage by weight |
|--------------------|----------------------|
| $TiO_2$ -----      | 94.8                 |
| $Fe_2O_3$ -----    | 1.15                 |
| Undetermined ----- | 4.05                 |
|                    | 100.00               |

The 4.05% undetermined can be assumed to have been 55 the oxides of Table I in about the same proportions as in said table.

The rutile was a fine material the largest particles of which were of about 46 grit size, the remainder finer particles all the way down to particles of a few microns size. 60 The coke was fairly uniform in particle size being about the same size as grains of rice. The rutile and the coke were well mixed.

My assistants under my direction then prepared the furnace bottom as already described by charging it with 65 rutile and then laid down the graphite masses and built the graphite bridge which were four inches wide and about two inches deep. The two graphite electrodes were four inches in diameter.

The furnace was started under an electromotive force of 50 volts with a power input of 150 kw. giving an average of 3000 amperes. The furnace was fed as described until all of the five hundred pounds of charge (mix) had been fed thereto. I kept the blanket or cover of mix at about one inch. Of course this is an estimate since 70 the contents of the shell emits tremendous illumination

at the temperatures involved. This run took four hours and seventeen minutes.

The yield was thirty six pounds of titanium carbide having an analysis as follows.

Table IV

| Element: | Percentage by weight |
|----------|----------------------|
| Ti       | 75.84                |
| C        | 16.80                |
| Fe       | 0.31                 |
|          | 92.95                |

Of the 7.05% not accounted for, obviously with so little boron to begin with, there could be very little in the product. Also the temperature is above the decomposition point of boron carbide and above the boiling point of  $B_2O_3$ . There can be little nickel in the product for similar reasons. The silicon, aluminum, calcium and magnesium are largely eliminated since the temperature is above the boiling points of these elements and above the decomposition points of silicon carbide and aluminum carbide. I believe the calcium and magnesium were largely eliminated. The phosphorus, tin and sulphur content is certainly mostly eliminated because of their low boiling points and the instability of their compounds. This leaves the elements Cr, Nb, V, and Zr as well as the Ti, C and Fe. The charge probably picked up a small percentage of nitrogen. Also some oxygen probably was present in the 7.05 percent remainder.

The ingots, one under each graphite electrode, were roughly cylinders with cracks. Each ingot was broken up with sledges and then crushed to produce lumps of various sizes, many an inch or two in longest dimension. Whatever is done with this material after this point is no part of the present invention. The material, however, is well suited for the uses mentioned in the objects.

This run, besides producing thirty-six pounds of titanium carbide yielded 85 lbs. of sweepings and 107 lbs. of refuse making 192 lbs. of reclaim material useful for further production of TiC. Some of the titanium content was lost in dust. In a large scale operation a dust collector is used to recover most of the dust.

## EXAMPLE II

In this example the mass of the charge, the electromotive force, the power in kilowatts, the rutile, the kind of coke, the manner of feeding the furnace, were all the same as in Example I. However the proportion was .75 free carbon to the mass of the rutile giving 275 lbs. of rutile and 225 lbs. of pitch coke. The free carbon content of the coke was close to .89. This run took four hours and seventeen minutes also. The yield was 53 lbs. of titanium carbide having an analysis of:

Table V

| Element: | Percentage by weight |
|----------|----------------------|
| Ti       | 71.47                |
| C        | 24.10                |
| Fe       | 0.31                 |
|          | 95.88                |

The balance of 4.12% probably involved the elements mentioned in the discussion of Table IV. Quantitatively there was probably considerably less oxygen in the material of Example II than there was in the material of Table IV (Example I). The ingots were broken up and crushed as in the case of Example I. This TiC was better grade material than that of Table IV for the uses mentioned in the objects since more of the oxygen was eliminated. The percentage of Ti in TiC is 80 and the percentage of carbon therein is therefore 20. It is noted that for the purposes indicated in the objects excess of carbon is not detrimental since, in the production of titanium metal by electrolysis in a fused salt bath the carbon will not deposit on the cathode.

In this run the sweepings weighed 67 lbs., the refuse weighed 104 lbs. making a total of 171 lbs. of reclaim material for subsequent use.

## EXAMPLE III

In this example the mass of the charge, the electromotive force, the power in kilowatts, the rutile, the kind of coke, the manner of feeding, the furnace, were all the same as in Examples I and II. However the proportion was .90 free carbon to the mass of the rutile giving 250 lbs. of rutile and 250 lbs. of pitch coke. The free carbon content of the coke was close to .9. This run took four hours and fifty-five minutes. The yield was 58 lbs. of titanium carbide having an analysis of:

Table VI

| Element: | Percentage by weight |
|----------|----------------------|
| Ti       | 69.37                |
| C        | 27.19                |
| Fe       | 0.14                 |
|          | 96.70                |

This product had less oxygen than those of Example I and II because there was 96.56% total titanium and carbon as compared with 95.57% for Example II, Table V and 92.64% for Example I, Table IV. Probably this product contained elements such as Cr, Nb, V and Zr in about the same relative proportions undetermined as in the cases of Examples I and II. The ingots were broken up and crushed as in the case of the other examples providing the best grade material for the uses mentioned. In this run the sweepings weighed 72 lbs., the refuse weighed 90 lbs., making a total of 162 lbs. of reclaim material for subsequent use.

## EXAMPLE IV

I have also made a run using an amount of coke to yield free carbon which was only the theoretical amount required to reduce the titania to titanium carbide, to wit, .45 times the amount of  $TiO_2$  which again I took to be the total mass of the rutile. The same rutile (Table III) was used and the same pitch coke having 88.7% free carbon. The mass of the charge, the electromotive force, the power in kilowatts and the manner of feeding the furnace were all of them the same as in the preceding examples. The charge was 335 lbs. of rutile and 170 lbs. of coke. This run took three hours and five minutes. The yield was 23 lbs. of titanium carbide analyzing:

Table VII

| Element: | Percentage by weight |
|----------|----------------------|
| Ti       | 79.38                |
| C        | 7.70                 |
| Fe       | 0.56                 |
|          | 87.64                |

This material is also believed to be useful for the extraction of titanium metal for example by chlorination. There is in the material of Example IV some suboxides of titanium, such as  $TiO$  and  $Ti_2O$ . The reaction of chlorine with TiC is exothermic while the reaction of the oxides of titanium with chlorine is endothermic. By using this material containing the carbide and some oxides of titanium the reaction with chlorine to produce titanium tetrachloride  $TiCl_4$  can be more closely controlled. The process for the extraction of titanium from its tetrachloride is known.

This material is further calculated to consist of:

Table VIII

| Material:          | Percentage by weight |
|--------------------|----------------------|
| $TiC + Fe$         | 38                   |
| $TiO_x$ and undet. | 62                   |
|                    | 100                  |

One of the especial features of the present process is having an electrically conductive path for the current between the arcs consisting of two ingots of titanium carbide separately formed under the electrodes plus the graphite bridge underneath the ingots. When finally the furnace has been filled with mixture to the brim, the power is cut off and the electrodes are raised. Of course the cascade of water was flowing over the furnace shell 20 at all times during the run of the process.

Another feature of the invention is the layer of rutile or reclaim material below the graphite or carbon bridge. This serves as an insulating layer to prevent short circuiting of the electric current path.

With regard to the electrical parameters, I have not found it practical to use higher than 150 volts and under 50 volts it is difficult to make a satisfactory product in reasonable quantity.

The important parameters in this invention are the parameters of the electromotive force, the proportion of free carbon in the mix and the parameters of the bridge. With regard to the latter, the cross section of the bridge is the criterion, since the bridge length is simply determined by the fact that it extends from under one electrode to under the other electrode, referred to as the loci of the electrodes.

The important feature of the cross section of the bridge is its area since the shape can vary widely within reason. This area is given as a function of the electrode diameter as I know of no other practical way to state it. The electrode diameter can be almost anything depending upon the size of the furnace. If the electrode is square, triangular or some other shape in cross section its "diameter" is taken as a function of its area A as if it were a circle. The diameter D of any circle is equal to

$$2\sqrt{\frac{A}{\pi}}$$

and for any figure the effective diameter D can be found by the equation

$$D = 2\sqrt{\frac{A}{\pi}}$$

Now if D is the diameter of the electrodes and C is the area of the cross section of the bridge in inches and square inches respectively, I find that the minimum value of C/D is 2 and the maximum value of C/D is 12. Thus I can state the bridge cross section by the formulae

$$C/D < 2 \text{ and } C/D > 12$$

In the practice of my invention I prefer to use the oval shell and two electrodes with single phase power. However three phase power could be used with three electrodes and then the shell should be trilobed or round.

The arc furnace process described, synthesizing titanium carbide, consumes far less pounds of electrode for every pound of production than does the resistance furnace process of the patent to Ridgway, No. 2,237,503. I do not have exact figures but am confident that the electrode consumption of my arc furnace process is less than one-tenth of that of the resistance furnace process per unit of product. Also my arc furnace process uses substantially less power per unit of production than does the resistance furnace process of Patent No. 2,237,503. Furthermore the production rate of my arc furnace process is much greater than that of the resistance furnace process.

The furnace shell 20, the table 65 and the oval bottom container 67 are stated to be made of steel. Steel is a variety of iron and other varieties of iron could be used, and also other metals could be substituted. Mixtures of two or more of the refractory materials alumina, titania and zirconia could be used for the furnace bottom under the carbonaceous bridge. The electrodes used were cylindrical in shape, but rod like electrodes of non-

circular cross section could be used. The ends of the graphite bridge covered the entire areas under the areas of the electrodes and this is preferable.

The process of the invention described herein is surprising when it is considered that the melting point of titanium carbide is 3140° C. while the boiling point of titanium metal is 3000° C. As there is no lid on the furnace one could expect the material to boil off when it has been reduced to the elemental stage. For it is obvious that you cannot go from  $TiO_2$  to  $TiC$  without passing through the stage  $Ti$ . As a matter of fact there are many stages or steps in the process going down (reducing) from  $TiO_2$  to  $TiC$ . We have:

TABLE IX

|    | Name                 | Formula            | Decomposes at |
|----|----------------------|--------------------|---------------|
| 20 | Titanium Dioxide     | $TiO_2$            | 1,640         |
|    | Titanium Sesquioxide | $Ti_2O_3$          | 2,130         |
|    | Titanium Monoxide    | $TiO$              |               |
|    | Titanium Suboxide    | $Ti_3O_2$          |               |
|    | Dititanium Oxide     | $Ti_2O$            |               |
|    | Titanium             | $Ti$               |               |
|    | Titanium Carbide     | $TiC$ , B.P. 4,300 |               |

25 Figures are degrees centigrade, B.P. = boiling point.

When  $TiO_2$  decomposes it goes to a lower oxide and the same is true for  $Ti_2O_3$ . I believe the lower oxides do not decompose to still lower oxides or to the metal because if so I would not need to add so much carbon. One, two or all of  $TiO$ ,  $Ti_3O_2$  and  $Ti_2O$  have a boiling point well below 3000° C., as calculated by thermodynamics, so it is surprising that  $TiC$  can be synthesized in the manner described.

30 35 By free carbon I mean available carbon, that is carbon available for reduction as distinguished from carbon in the hydrocarbon content, etc.; sometimes free carbon is called fixed carbon. Since graphite is a form of carbon and since amorphous carbon can be used for the bridge as well as graphite, in the claims the expression "bridge of carbon" or the like is to be construed as covering a bridge of graphite or a bridge of amorphous carbon.

40 45 In the patent to R. R. Ridgway, No. 2,285,837, a process of producing carbides, including titanium carbide, in an arc furnace is described. In this Ridgway process a molten pool of the carbide is formed, as shown in the drawings and as stated on page 3, left hand column, line 9. This was found to cause reoxidation of the carbide resulting in a low grade product. The theory that the use of a deep furnace would avoid oxidization and nitriding was valid only in part. By avoiding the formation of any substantial pool of molten carbide, the process herein described is a much more practical arc furnace method of making titanium carbide and produces a better product.

50 55 Further details of the operating conditions for a furnace of the size illustrated and described which also hold for furnaces of about the same size with electrodes approximately as described are as follows:

60 The first adjustment to be made when the furnace is ready to start is to set the voltage at a suitable value. The range of voltages that can be used with the furnace noted above is from 50 to 150 volts; the recommended value for best operation being 100 volts. The adjustment is the current level. The current controller raises or lowers the electrodes automatically to maintain a predetermined current. The range of currents that can be used is from 4,000 to 10,000 amperes, the optimum value being 8,000 amperes. Under optimum conditions, this size and type of furnace therefore runs at 100 volts and 8,000 amperes, corresponding to a total input of 800 kva. This type of furnace runs at a power factor sufficiently close to unity for us to speak of kva. and kw. interchangeably, so I shall call this 800 kw.

65 70 75 The ranges of voltage and current noted above still do not specify completely the possible operating conditions.

For example 150 volts at 10,000 amperes would cause erratic furnace operation while 50 volts and 4,000 amperes would reduce the rate of production to an uneconomically low level. A further limitation must therefore be placed on the operation, restricting the power level to the range from 350 to 1000 kw. FIGURE 13 shows graphically the permissible operating conditions.

The discussion above describes a comparatively wide range of power levels, roughly three to one. It is to be expected that the resulting product will differ in some respects, depending on the particular set of operating conditions selected, and this expectation is borne out by experience. For one thing, the power level will determine the diameter of the twin ingots that grow in the furnace. Thus, at the lower limit of 350 kw. the ingots will be about 14 inches in diameter, and at the upper limit of 1000 kw. they can be up to 24 inches in diameter. Since the electrodes are spaced 24 inches center to center, the latter figures represent a limiting condition under which the ingots begin to touch each other at some points. For another thing, the power level will influence the rate at which the ingots grow vertically. However, this rate of growth is taken care of automatically providing the raw materials are fed to the furnace at the specified rate, which I shall now discuss.

Probably the most important single consideration in the operation of the furnace is the control of the process of reaction and incipient fusion that makes it possible to grow ingots without at any time forming a molten pool of product in the bottom of the furnace. This process is controlled by feeding the raw materials to the furnace at a predetermined rate. Thus the feed rate must be held between 0.5 and 0.75 lb. of raw mix per kwh. As an example, if the furnace is run at a power level of 1,000 kw., the total energy used in one hour is 1000 kwh. It will therefore be necessary to feed the raw mix to the furnace at a rate between 500 and 750 lb. per hour. Since by no means all the feed is reacted in any one run, the overall consumption of electrical energy by the process is 4-8 kwh. per lb. of product.

It will thus be seen that there are as many distinct ingots of titanium carbide as there are electrodes, and that the ingots are maintained substantially clear of each other so that the major path of the electric current after the process has been started is from one electrode to another electrode, via first an electric arc between an electrode and the titanium carbide ingot under it, then through a mass of carbon, then through the bridge, then through another carbon mass, then through another titanium carbide ingot and finally through an electric arc to the electrode directly above the ingot.

It will thus be seen that there has been provided by this invention a process for the production of titanium carbide in which the various objects hereinbefore set forth, together with many thoroughly practical advantages are successfully achieved. As many possible em-

bodiments may be made of the above invention and as the art herein described might be varied parts, all without departing from the scope of the invention, it is to be understood that all matter hereinabove set forth or shown in the accompanying drawings is to be interpreted as illustrative and not in a limiting sense.

I claim:

1. The process of synthesizing titanium carbide by the reaction of titanium oxide ore and coke in an electric arc furnace while maintaining reducing conditions at the zones of reaction, which comprises forming in an electric arc furnace having vertically movable electrodes a furnace bottom of refractory oxide material, placing a mass of carbon above said bottom at the eventual locus of each electrode, forming a bridge of carbon above said bottom electrically connecting said masses, maintaining said bridge of carbon at all times during the process, placing said electrodes at said loci in electrical contact with said masses of carbon and energizing said electrodes at from 10 50 to 150 volts, maintaining during the process a mixture of said titanium oxide ore and coke around the bottoms of said electrodes and forming thereby as many distinct 15 ingots of titanium carbide as there are electrodes one ingot under each electrode, feeding said mixture of titanium oxide and coke to around the bottoms of said electrodes from 20 at the rate of from 0.5 to 0.75 lb. of mixture per kwh. of electrical energy energizing said electrodes, and maintaining the said ingots clear of each other whereby the 25 path of the electric current after the process has been started is always from one electrode to another electrode, via first an arc, then through a titanium carbide ingot synthesized by the process, then through one of said masses of carbon, then through the bridge, then through another of said masses of carbon, then through another titanium carbide ingot synthesized by the process, then by 30 an arc to another electrode, and building up the titanium carbide ingots synthesized by the process under the electrodes without the formation of any considerable pool of molten titanium carbide as the electrodes gradually rise 35 during the process by reason of the energization of the electrodes at 1 kwh. for each 0.5 to 0.75 lb. of mixture fed.
2. Process according to claim 1 in which the cross section of the bridge in square inches divided by the diameter 40 of the electrode in inches is between 2 and 12.
3. Process according to claim 2 in which the oxide material of the furnace bottom is mainly titanium oxide.
4. Process according to claim 1 in which the oxide 45 material of the furnace bottom is mainly titanium oxide.

#### References Cited by the Examiner

##### UNITED STATES PATENTS

- |              |      |         |        |
|--------------|------|---------|--------|
| 2,237,503    | 4/41 | Ridgway | 23—208 |
| 55 2,285,837 | 6/42 | Ridgway | 23—208 |

MAURICE A. BRINDISI, Primary Examiner.